

## UNITED STATES PATENT OFFICE

2,316,220

## COMPOSITION FOR CLEANING ALUMINUM

Robert H. Brown, New Kensington, and Robert B. Mears, Oakmont, Pa., assignors to Aluminum Company of America, Pittsburgh, Pa., a corporation of Pennsylvania

No Drawing. Application April 22, 1939,  
Serial No. 269,489

4 Claims. (Cl. 252—136)

This invention relates to an improved cleaning agent. More particularly, it relates to a non-abrasive acid cleaning composition which may be packaged in dry form and dissolved in water for use.

While cleaning compositions having acid reactions are known in the art, most of them are liquid in form. For that reason, they require careful handling and must be packaged in the more expensive containers designed to hold such substances; these containers may be broken during shipping or handling, and great damage may then be caused by their acid contents. Moreover, such liquid acid compositions occupy substantial storing space.

The object of this invention is to provide a novel cleaning composition in dry or solid form which may easily be handled and packaged. More particularly, the object is to provide such a composition having an acid reaction. The specific object of the invention is to provide a non-abrasive cleaning composition which may be packaged in dry form and used in an aqueous solution for cleaning the surfaces of aluminum or aluminum alloy articles. Other objects will appear in the following description of the invention.

We have found that stains and discolorations are very readily removed from the surfaces of articles by immersing said articles in a hot aqueous solution containing an alkali metal acid phosphate in suitable concentration, depending upon the nature of the articles being cleaned. These phosphates are all solid and may be packaged in powdered or in granular form until ready for use. Then, since they are all water-soluble, they may be dissolved in water at a temperature near its boiling point to provide a cleaning medium which is sufficiently acid in reaction to be effective, yet not so violent as to attack and mar the surfaces of the articles being cleaned. The alkali metal acid phosphates have particular value in the cleaning of aluminum or its alloys, and are particularly effective in removing discolorations from the surfaces of aluminum kitchen utensils, barrels, dairy equipment, and other articles of aluminum or aluminum alloy.

Although sodium, potassium, and other alkali metal phosphates having an acid reaction are effective for cleaning tarnished surfaces of aluminum articles, we prefer to use ammonium dihydrogen phosphate, which is included in the classification of an "alkali metal acid phosphate." This compound is inexpensive and readily available, and it appears to be more strongly

acid than the other alkali metal acid phosphates.

While all of the alkali metal acid phosphates are individually sufficiently active to remove discoloration from the surfaces of aluminum and other articles, it may be desired to increase their effectiveness in this respect. This may be done by using with them an additional substance adapted to increase the acid reaction of the aqueous alkali phosphate solution. The additional substance also should be solid in form in order that it may be packaged with the alkali phosphate, and it should be soluble in water so that it may be dissolved in the aqueous phosphate solution. We prefer to use an alkali metal acid sulfate, such as ammonium bisulfate, as the additional acid substance; other acids or acid salts also may be used to advantage, among them being metaphosphoric acid, sulfamic acid, and the alkali metal fluorides, ammonium bifluoride being especially effective. A cleaning composition containing an alkali metal acid phosphate and sulfamic acid is claimed in our copending application Serial No. 269,490, filed April 22, 1939. In addition, we have found that tartaric acid may be used with this additional substance where it is desirable that the cleaning solution should work with even greater effect. Tartaric acid also is solid and water-soluble, and may be packaged in dry form with the alkali metal phosphate and any of the substances above named.

Instead of using a substance with the alkali metal acid phosphate which increases the acidity of the solution, the additional solid, water-soluble substance may be a neutral compound capable of dissolving in the aqueous phosphate solution and reacting in water to form an acid which will etch the particular material being cleaned. For example, in the cleaning of aluminum, sodium fluoride in the phosphate cleaning composition dissolves in water to form hydrofluoric acid, which supplements the cleaning effect of the acid phosphate.

The addition of wetting agents, such as certain of the alkyl sulfonates, also may be profitable, since cleaning may be effected in their presence with a smaller amount of phosphate and additional substances in the solution. The particular wetting agent used should be determined by the nature of the object being cleaned.

In the practice of one embodiment of the invention, we have used 25 grams of ammonium dihydrogen phosphate and 25 grams of ammonium bisulfate dissolved in one liter of water, the solution being heated to near 100° C. This solu-

tion removes the discoloration from aluminum articles very readily. The time during which the articles are immersed in the solution depends upon the extent to which their surfaces are tarnished, but in most cases a 5-minute treatment results in the removal of all stains and leaves their surfaces clean with a slightly frosted appearance.

Although the invention has been described with reference to the cleaning of aluminum, and although it has particular value when used for removing discoloration from the surfaces of that metal, it may be employed for cleaning other materials as well.

We claim:

1. A process for cleaning the surfaces of articles of aluminum, which comprises subjecting said surfaces to the action of a hot aqueous solution of a composition consisting substantially of an alkali metal fluoride and ammonium dihydrogen phosphate, the latter being the major component and the principal active cleansing agent.

2. A dry water-soluble aluminum-surface

cleanser for use in aqueous solution, said cleanser being characterized by an acidic cleansing reaction in said solution and consisting substantially of an alkali metal fluoride and ammonium dihydrogen phosphate, the latter being the major component and the principal active cleansing agent.

3. A dry water-soluble aluminum-surface cleanser for use in aqueous solution, said cleanser being characterized by an acidic cleansing reaction in said solution and consisting substantially of sodium fluoride and ammonium dihydrogen phosphate, the latter being the major component and the principal active cleansing agent.

15 4. A dry water-soluble aluminum-surface cleanser for use in aqueous solution, said cleanser being characterized by an acidic cleansing reaction in said solution and consisting substantially of an alkali metal fluoride and an alkali metal acid phosphate, the latter being the major component and the principal active cleansing agent.

ROBERT H. BROWN.

ROBERT B. MEARS.